

June 12, 1945.

J. R. CALDWELL  
RESILIENT SYNTHETIC YARN

2,378,183

Filed Oct. 9, 1941

STRESS-STRAIN CURVE

Fig.1



RESILIENCY CURVE

Fig.2



John R. Caldwell  
INVENTOR

BY *Nelson M. Brooks*  
*Daniel J. Mayne*  
ATTORNEYS

## UNITED STATES PATENT OFFICE

2,378,183

## RESILIENT SYNTHETIC YARN

John R. Caldwell, Kingsport, Tenn., assignor to  
 Eastman Kodak Company, Rochester, N. Y., a  
 corporation of New Jersey

Application October 9, 1941, Serial No. 414,265

4 Claims. (Cl. 260—14)

This invention relates to the preparation of synthetic yarns having special physical and mechanical properties and more particularly to the preparation of wool-like, resilient yarns composed of or containing cellulose derivatives, such as cellulose organic acid esters, such as cellulose acetate, cellulose acetate propionate and the like, and the cellulose ethers.

As is well known, yarns and fibers produced from synthetic materials such as viscose, cellulose derivatives and resins differ in many respects from natural products such as silk, cotton, wool and the like. It is also known that synthetic yarns differ widely among themselves in physical and chemical properties, some having certain inherent characteristics which make them particularly well adapted for certain uses, while other yarns have characteristics which render them unsuitable for such uses. From the earliest beginnings of the synthetic yarn industry, research has constantly been going on with the object of so modifying such artificial materials as more closely to simulate or duplicate the valuable properties of natural fibers. To the credit of the research workers in this field, it may be said that in many instances, not only have the properties of natural fibers been duplicated in synthetic yarns, but actually have been improved upon. On the other hand, it has been found impossible to duplicate certain other properties in synthetic yarns.

The difficulties involved in dealing with synthetic materials produced from cellulose derivatives, such as cellulose acetate and similar cellulose organic acid esters, as well as the cellulose ethers, are multiplied because of the plastic or semi-plastic nature of the material and its susceptibility to cold flow. In general, it may be said that to attain any given property or combination of properties in such a yarn, it is always necessary to balance a number of factors one against the other. For example, it may in a given instance be quite easy to produce a yarn having high tensile strength and other desirable properties and at the same time fail to attain the desired degree of stretch or stretchability of the yarn to make it a practical commercial product. Likewise, it may be a relatively simple matter to crimp a cellulose derivative yarn by various mechanical means or to give it certain surface irregularities simulating natural wool and yet not arrive at a product which will retain its crimp or possess the springy, resilient hand or feel of natural wool fibers.

An immense amount of research has gone into

the problem of producing a satisfactory type of synthetic yarn or fiber which will have most of the desirable characteristics of natural wool. This is particularly true of attempts to obtain a cellulose derivative yarn which will possess high crimp retentivity and springiness and will at the same time be susceptible of crimping by mechanical means under the influence of heat and pressure without otherwise being adversely affected. 5 In recent years, literally hundreds of attempts have been made to solve this problem and the patent and technical literature contains a multitude of references to the use of various and sundry expedients. One of the most common of 10 these expedients is to impregnate a preformed yarn with a solution of a resin. Included among the resins suggested for the purpose are the so-called heat-hardening resins such as those obtained by condensing phenol and formaldehyde, urea and formaldehyde and others. Another suggestion has been to incorporate such resins or solutions of resins in the spinning solution from which the yarn is produced. In either case the yarn containing the resin or resin-forming 15 components is subjected to some sort of physical or chemical treatment which brings about hardening of the resin, as for example, a heat treatment, the theory being that since the resinous material sets under the influence of heat, the yarn will be stiffened and thus rendered resilient. 20

Notwithstanding the many expedients suggested for the production of this type of yarn, none of them, to the best of my knowledge and belief, 25 has offered a complete solution of the problem. While synthetic yarns have heretofore undoubtedly been stiffened by impregnation with, or by formation in situ of, heat-hardening resins in the manner just referred to, it appears that in 30 no instance have all of the various factors necessary for the production of a satisfactory commercial yarn of this type been so balanced or coordinated as to give the desired product. Presumably, this has been due to a failure upon the part of research workers in this field fully to appreciate the theoretical considerations involved. In order more fully to explain the advance in the 35 synthetic yarn art represented by the present invention, this matter of theory will now be briefly adverted to.

As indicated above, it may be said that, in general, fibers prepared from derivatives of cellulose typified by cellulose acetate, cellulose acetate propionate and the like, possess relatively little elasticity as compared to natural fibers such

as silk and wool. For example, if natural silk is stretched to an elongation of approximately 10% and subsequently released, it will return substantially to its original length. If a cellulose acetate fiber, on the other hand, is subjected to the same treatment, it shows very little tendency toward recovery and will remain permanently elongated. This permanent elongation is due to plastic flow, a property inherent in the structure of all cellulose esters to a greater or less extent. 10 To employ the language of mechanics, these materials have a relatively low yield point, this term being defined as that point on the stress-strain curve where relatively small increments in the magnitude of applied force or stress cause large 15 changes in elongation or strain. Another way of defining yield point is as that section of the stress strain curve in which the slope undergoes the greatest rate of change. Numerous physical tests, as well as data obtained from other sources such as X-ray diagrams and the like, demonstrate the fact that cellulose ester yarns belong to the 20 class of non-elastic substances, that is, they show a well-defined yield point and readily undergo permanent deformation.

The molecular or structural units or micelles of which cellulose derivative fibers are composed have relatively low cohesive forces. Furthermore, they are of such nature that under conditions of stress, these molecular units slide past 30 each other and assume new permanent positions when the stress or applied force is released. These slippage planes or areas of relatively low cohesive force contribute in a considerable degree to the relatively large permanent deformation observed in cellulose derivative fibers.

As will be more fully explained by reference to specific examples appearing hereinafter, I have found that the yield point characteristics of a cellulose derivative fiber are closely associated with the properties of stiffness and resiliency. Textile materials possessing these properties are described as having a wiry or springy hand or feel. Wool is a good example of a natural product having such properties. For example, if a mass of wool fiber is compressed and then released, it will spring back almost immediately to substantially its original volume. It is this characteristic which gives woolen fabrics their strength and wearing qualities. An analysis of the stress-strain curve for wool shows that there is no well defined yield point as found in the case of cellulose acetate or other cellulose derivative synthetic fibers. Hence, it must be concluded that the closer the stress-strain curve of such synthetic fibers approaches that of wool, the closer will be the resemblance of the synthetic product to the natural product as to resiliency, elasticity and similar properties.

This invention has as an object to provide a cellulose derivative yarn or fiber having resiliency, elasticity and other properties comparable to wool and other natural fibers. A further object is to provide a cellulose acetate or other cellulose derivative yarn which is susceptible of permanent mechanical crimping or other deformation without the loss of any of the yarn's desirable physical properties. A still further object is to provide a process of preparing a springy, resilient, elastic cellulose derivative yarn or fiber of the type specified. A specific object is to improve upon known processes of producing resin-containing synthetic yarns and to obtain a product possessing properties superior to those of known synthetic yarns. Other objects will appear hereinafter.

These objects are accomplished by the following invention which, in its broader aspects, comprises combining with a cellulose derivative yarn as an integral part of the internal structure of the yarn material itself, a specific type of thermosetting resin in certain specific proportions and under such conditions that a permanently resilient yarn will be obtained. It is desired particularly to point out that the resin after formation under carefully controlled conditions is added to the spinning solution and thus is incorporated in the yarn structure itself, as differentiated from impregnation of a preformed yarn with the resin.

It should be noted at this point that the present invention involves the use of a very special type of resin which must meet certain specific requirements. After an extensive investigation I have found that in order to meet such requirements, the resin must have the following characteristics: (a) it must be soluble in acetone or whatever solvent is employed for dissolving the cellulose ester in making up the spinning solution, (b) it must be compatible with the cellulose ester in the dope, (c) it must be chemically inert toward the cellulose ester, (d) it must be compatible with the cellulose ester when the solvent is evaporated, (e) it must be sufficiently light in color to avoid discoloring the yarn, (f) it must be convertible to a form which will be resistant to washing, ironing and other textile processing treatments, (g) it must be thermosetting under such conditions of time and temperature as will not injure the cellulose ester fiber and (h) it must be capable of forming a continuous rigid structure in the yarn which exerts a stiffening and reinforcing action throughout the body of the material.

As will be readily appreciated, many resins fall short in one or more respects of meeting the above specifications. In fact, in carrying out research on this problem, I have investigated phenol-formaldehyde- and urea-formaldehyde resins, the so-called alkyd resins of the phthalic anhydride-polyhydric alcohol type, polymeric derivatives of acrylic acid, polymeric derivatives of vinyl acetate and vinyl chloride and resins derived from drying oils. All of these classes of resins were found deficient in one or more of the essential requirements. For example, many alkyd resins showed excellent compatibility but required excessively high temperatures for curing. Phenol formaldehyde resins were satisfactory from the standpoint of compatibility and curing temperature but lacked sufficient reinforcing action. Urea formaldehyde resins cured rapidly to hard, tough products, but tended to be incompatible with the cellulose ester material.

After many experiments were carried out, I found that a resin condensation product formed by the interaction of phenol, urea and formaldehyde under carefully controlled conditions met each and every one of the above requirements and made possible the production of a superior yarn product having the desired qualities of springiness, resiliency, elasticity and the like. The resin condensation products contemplated by my invention may be defined as products formed by condensing in aqueous medium and under alkaline conditions the following components:

(a) One mol proportion phenol or alkyl substituted phenol containing at least two free active positions on the nucleus; An active position being defined as ortho or para to the hydroxyl group, (b) from 0.15 to 1.0 molar proportions

urea, thiourea, or mono-N-substituted urea or thiourea, (c) 3 to 5 molecular proportions of formaldehyde.

In addition to phenol many types of alkyl substituted phenol derivatives having two free active groups are suitable for the process, for example: ortho-, para-, or meta-cresol; 1,3,5 xylenol; p-tertiary butyl phenol; 2-ethyl phenol, etc. For economic reasons it is sometimes preferable to use a mixture of substituted phenols, as for example, the commercial mixture of meta- and para-cresol. Resins with improved color characteristics are obtained if the phenols are distilled just prior to use.

Although the best resins are produced with urea or thiourea, it is possible to use N-substituted ureas as for example N-butyl urea, N-ethyl urea, etc. Formaldehyde may be employed in the form of 40% formalin or as an aqueous suspension of paraformaldehyde. The reaction is carried out within a temperature range from 70° C. up to the atmospheric pressure boiling point of the reaction mixture.

Suitable resins are formed only under alkaline conditions, and I have found that amines are superior to mineral alkalis as catalysts, although either may be used. Among typical amine catalysts may be mentioned ammonia, mono-, di-, and trimethyl amine, the corresponding ethyl amines, pyridine, higher amines such as butyl amines, amyl amines and similar amines. I have found that the type of catalyst employed exerts a profound influence upon the properties of the resin. Among the catalysts just referred to, a mixture of monobutylamine and ammonia proved to be a highly specific catalyst that gave resins considerably superior to those made with other alkalis. In carrying out the condensation reaction a sufficient amount of the catalyst is added at the beginning to maintain a pH value of 7.5-9.5 throughout the entire course of the reaction.

The time of reaction varies considerably with the nature and proportions of the components. For example: meta-cresol will react faster than the para derivative. In general, the condensation is carried to a point where the product is soluble in acetone and curable in three to four hours at 100°-125° C. This point can be determined only by trial and error because of the many variables which influence the reaction rate.

In employing the resin for the manufacture of a resilient type of yarn in accordance with my invention, anywhere from 5-30% and preferably 10-20% of the resin based on the weight of the cellulose ester, may be employed.

As will be more fully set forth hereinafter, the resin-bearing yarn is cured at an appropriate temperature. In general, the most practical curing temperature is within the range of 90-125° C. At this temperature, curing takes place in 1-3 hours depending upon the nature of the specific resin used. Curing will take place more rapidly at temperatures above 125° C. but there is danger of discoloring or tendering the yarn. In some cases, as with resins containing an appreciable amount of meta cresol, a curing temperature of 70-80° C. is suitable. The optimum curing range of temperature and time must be determined separately for each resin type because of individual differences in reactivity.

I wish to particularly point out that only resins prepared in accordance with the above description meet each and every one of the eight essential requirements of a resin to give an actual

ly springy, resilient yarn when employed in accordance with the invention. It is desired to emphasize the fact that each of these requirements must be met and that deficiency in a single one immediately eliminates the resin from consideration. It is thus evident that a resin suitable for the purposes outlined herein is a highly specific composition possessing well-defined and closely-restricted properties and cannot be obtained by merely selecting at random from the numerous resins of the prior art.

In the following examples and description, I have set forth several of the preferred embodiments of my invention, but they are included merely for purposes of illustration and not as a limitation thereof.

In the accompanying drawing:

Fig. 1 is a graph illustrating the stress-strain curve of a cellulose organic acid ester yarn which has been treated, both in accordance with the invention, and without such treatment.

Fig. 2 is a graphical representation of the resiliency of a cellulose organic acid ester yarn, both with and without, a resin employed in accordance with the invention.

#### Example 1

A mixture having the following composition:

|                                           | Parts by weight |
|-------------------------------------------|-----------------|
| Mixed meta- and para-cresols              | 25              |
| Urea                                      | 8               |
| (40% aqueous solution) formaldehyde       | 90              |
| (28% aqueous solution) ammonium hydroxide | 8               |

is heated to boiling under reflux and maintained at this temperature for twenty to thirty minutes. Part of the resin separates as a viscous syrup which settles to the bottom of the reaction vessel. The mixture is then evaporated at reduced pressure to a water content of 25%-35% as determined by distillation with toluene. The final product is a viscous syrup soluble in acetone. For convenience in handling, the resin is dissolved in acetone to form a 30%-60% solution.

For preparation of the yarn, a spinning solution or dope is prepared having the following composition:

|                   | Parts by weight |
|-------------------|-----------------|
| Cellulose acetate | 25              |
| Acetone           | 72              |
| Resin             | 3               |

I have found that it is often advantageous to employ a curing catalyst with the resins. The catalyst may be incorporated in the resin solution prior to mixing with the spinning dope, or it may be added directly to the spinning dope. Salts formed by reacting certain amines with weak acids are well suited as catalysts. Among these may be mentioned butylamine propionate, morpholine acetate, amylamine acetate and morpholine borate. The catalyst is added to the extent of 1%-5% based on the weight of the resin. For this particular resin, 2% morpholine acetate is used as catalyst.

A dope prepared as just described is extruded into an evaporative atmosphere (dry spinning) or precipitating bath (wet spinning) by known methods, as, for example, the processes described in the U. S. patents to Stone 2,000,048 and 2,000,049, and wound onto a suitable package.

The yarn so formed is then heated at a temperature of 90°-130° C. from one to five hours to cure the resin. It may be heated in the form

of skeins, or on spools, bobbins, etc. It is often advantageous to use bobbins or spools with perforated cores to promote circulation of air.

Yarn prepared according to this method has a relatively high yield point and possesses improved elastic properties. In Fig. 1 of the drawing the stress-strain curve illustrates the influence of the resin on the elastic properties of the yarn. Curve A is that obtained by testing a cellulose acetate yarn prepared as described above and containing 10% of the resin in accordance with the invention. Curve B is for a similar yarn but containing no resin. It will be observed that the yield point Y for yarn containing the resin is 1.00 gram per denier while the yield point Y' for the yarn containing no resin is 0.72 gram per denier. Thus the use of resin gives rise to an improvement of 39%. It is therefore evident that the presence of the 10% of this particular resin has imparted new and valuable properties to the fiber. Incidentally, it will be observed that the stretch has been somewhat reduced.

The fiber produced as described in the preceding paragraphs may be processed on the usual weaving and knitting machinery to give fabrics having excellent fullness of hand. Fabrics prepared from yarn of this type show superior elastic properties and excellent resistance to stretching and sagging. It is notable that many of the resins falling within the scope of my invention raise the melting and/or softening point of the yarn. For example, the melting point of the fiber just described is 260°-262° C., whereas the yarn without the resin has a melting point of 250°-252°. This is also an important characteristic of my invention, the net effect of which is to raise the safe ironing point of a fabric made from such yarn.

#### Example 2

A mixture having the following composition

Parts by weight

|                 |     |
|-----------------|-----|
| Phenol          | 15  |
| 1,3,5 xylene    | 15  |
| Thiourea        | 10  |
| Formalin (40%)  | 100 |
| Monomethylamine | 1   |

is heated under reflux at 100° C. over a water bath for one hour, after which it is concentrated by vacuum distillation to a water content of 24-35%. The mixture is then incorporated in the spinning dope as described in Example 1 and spun into yarn according to standard procedure. As a curing catalyst, 3% butylamine propionate is employed.

#### Example 3

In some cases it may be desirable to prepare resins employing a mixture of urea and thiourea, for example. A mixture having the following composition

Parts by weight

|                  |    |
|------------------|----|
| Urea             | 8  |
| Thiourea         | 8  |
| Mixed m-p-cresol | 25 |
| 40% formalin     | 90 |
| Diethylamine     | 1  |

is worked up by a procedure similar to that described in Examples 1 and 2 above. The resin thus produced is incorporated in a spinning solution and yarn spun therefrom in accordance with standard procedure. Following the heat treatment referred to in Example 1, the yarn is found

to have excellent properties of resiliency, fullness of hand.

#### Example 4

A resin having outstanding properties for use in a spinning solution as outlined in the preceding examples may be prepared from the following composition:

|                          |          |
|--------------------------|----------|
| Meta-para cresol         | grams 20 |
| Urea                     | do 10    |
| Formalin (40%)           | cc 90    |
| Conc. ammonium hydroxide | cc 5     |
| Monobutylamine           | cc 2     |

The mixture is boiled for 20 minutes, then evaporated under vacuum to a water content of 20%-30% as shown by boiling toluene extraction.

As will be apparent to those skilled in the art, the impregnated yarns of my invention are useful for many purposes. Because of the high yield point of the material, it is especially suitable for use in fabrics where resistance to crushing is desired, such as in carpets, blankets, velvets, upholstery and similar pile fabrics. It is of especial value in the preparation of cut staple fibers, particularly those which are to be employed as wool substitutes, because of the fact that the resin imparts an appreciable stiffness and elasticity to the yarn and thus gives it an especially resilient hand and a close resemblance to natural wool.

Staple fibers prepared in accordance with the present invention show a markedly improved permanence of crimp because of their high yield point, that is, a much greater load is required to remove the crimp and permanently straighten the fiber than is the case with ordinary yarns and with other resin-impregnated yarns. A product closely resembling natural wool may be produced by crimping cellulose acetate and other cellulose organic acid ester yarns, containing resins according to my invention, by the mechanical crimping process described in my copending application Ser. No. 366,887, filed November 23, 1940, and then subjecting the crimped and resin-impregnated yarn to a heat treatment to thermoset the contained resinous materials.

Other uses which the particular properties of my product make possible are as stuffing or filling for padded articles such as chair cushions, automobile seats and the like. Because of its close similarity to wool, the resin-bearing fiber material may also be employed in men's suiting, worsteds and similar fabrics.

As will be indicated by the curves of Figs. 1 and 2, yarn prepared in accordance with my invention and containing 10-20% of phenol-urea-formaldehyde resin gives rise to an appreciable improvement in the yield point of the yarn as compared to yarns not so treated and imparts a stiffer, more resilient feel to the material, thus increasing its resemblance to natural wool. Naturally, the stiffening process results in some loss of stretch, but this is relatively insignificant. I have found, for example, that when 10-20% of resin is employed in the yarn, it gives approximately a 40% increase in the yield point. Tests have shown that it takes 30-40 greater longitudinal stress to remove the crimp from yarn containing 10% resin as compared to normal yarn. Analysis of the stress-strain curve of Fig. 1 shows beyond all doubt that the resin sets up to a semi-rigid structure or skeleton within the body of the filament which imparts a pronounced stiffening action to the yarn and brings about a significant reduction in the cold flow tendency of the cellulose derivative material.

Referring to Fig. 1 curve A was plotted from data taken on yarn containing 10% phenol-urea-formaldehyde in accordance with my invention. The yield point is indicated by the letter Y. The stress-strain curve of the same yarn without the resin is illustrated by the curve B, the yield point of this yarn being indicated by the letter Y<sub>1</sub>. It will be seen that, not only does yarn A have a much higher yield point than yarn B, but that the shape of the stress-strain curve, especially in the vicinity of the yield point is profoundly altered by the presence of the resin.

The property of a fiber to spring back after deformation is best described by the term "resiliency." Wool is a typical example of a fiber which possesses resiliency to a high degree. This quality may be measured quantitatively and it is found that a cellulose acetate yarn prepared in accordance with my invention and containing 10-20% of a phenol-urea-formaldehyde resin is considerably more resilient than a similar yarn which does not contain the resin. Typical resiliency curves are shown in Fig. 2. These curves were obtained by plotting the amount of force necessary to compress a given weight of staple through the distance shown on the horizontal axis. The pressure was then gradually removed from the staple and it was allowed to recover. Each sample is represented by two curves, the one on the left showing compression, the one on the right showing expansion or recovery. The area enclosed by the two curves is inversely proportional to the resiliency or recovery tendency of the fiber. That is, if the fiber were perfectly elastic and returned completely to its original shape, the compression curve and expansion curves would coincide. The area enclosed between the two curves thus represents the energy lost by hysteresis, that is, the difference between the work done to compress the yarn and the work given back by the yarn during expansion.

It will be noted that the area enclosed by curves A plotted from data taken on a yarn containing a phenol-urea-formaldehyde resin in accordance with my invention, is considerably smaller than that enclosed by the curves B plotted from data taken on the same yarn containing no resin. This strikingly illustrates the superiority of the resin-containing yarn in its tendency to return to its original shape as compared to an ordinary yarn and shows that it is much more resilient.

It is particularly to be noted that the resins prepared as described above are, in accordance with my invention, added to the spinning solution and cannot be applied to preformed yarn. Thus, the present process is to be differentiated from previously known processes wherein preformed yarns, fibers or fabrics are soaked or impregnated with resin-forming materials. Although many proposals have been made for incorporating in a spinning solution a thermosetting resin or the components from which such a resin could be formed in situ, to the best of my knowledge and belief, no practical process for obtaining a resilient resin-impregnated yarn has ever before been suggested or disclosed in the prior art. Due to the fact that in the present process the resin is mixed with the spinning solution so that a homogeneous dispersion or solution thereof is obtained, the resin becomes an integral part of the fiber structure after the yarn is formed and thus exerts its reinforcing action throughout the entire cross-section of the filament.

What I claim is:

1. A synthetic yarn spinning solution comprising a cellulose organic acid ester dissolved in a volatile solvent and containing in solution 5-30%, based on the weight of the cellulose ester of a partially polymerized phenol-urea-formaldehyde resin prepared by condensing under alkaline conditions 1 molecular proportion of a phenol selected from the group consisting of phenol and alkyl-substituted phenols containing at least two free active positions on the nucleus with from 0.15 to 1.0 molecular proportion of a urea selected from the group consisting of urea and mono-N-alkyl substituted ureas and mono-N-alkyl substituted thioureas and 3-5 molecular proportions of formaldehyde, said resin being susceptible of further polymerization under the influence of heat, said resin in its further polymerized form having the property of imparting to yarn formed from said solution, a high degree of resiliency, elasticity, a springy hand or feel and a yield point in the neighborhood of 1 gram per denier.
2. A synthetic yarn spinning solution comprising a cellulose organic acid ester dissolved in a volatile solvent and containing in solution 5-30%, based on the weight of the cellulose ester of a partially polymerized phenol-urea-formaldehyde resin prepared by condensing 1 molecular proportion of a phenol selected from the group consisting of phenol and alkyl-substituted phenols containing at least two free active positions on the nucleus with from 0.15 to 1.0 molecular proportion of a urea selected from the group consisting of urea and mono-N-alkyl substituted ureas and mono-N-alkyl substituted thioureas and 3-5 molecular proportions of formaldehyde, in the presence of a mixture of monobutylamine and ammonium hydroxide as catalyst, said resin being susceptible of further polymerization under the influence of heat, said resin in its further polymerized form having the property of imparting to yarn formed from said solution, a high degree of resiliency, elasticity, a springy hand or feel and a yield point in the neighborhood of 1 gram per denier.
3. A synthetic yarn spinning solution comprising 25 parts by weight of cellulose acetate, 72 parts by weight acetone and 3 parts by weight of a phenol-urea-formaldehyde resin prepared by boiling for approximately 20 minutes a composition having the following components:

|                          |       |    |
|--------------------------|-------|----|
| Meta-para cresol         | grams | 20 |
| Urea                     | do    | 10 |
| Formalin (40%)           | cc    | 90 |
| Conc. ammonium hydroxide | cc    | 5  |
| Monobutylamine           | cc    | 2  |

and evaporating to a water content of 20-30%.

4. A synthetic yarn spinning solution comprising a cellulose organic acid ester dissolved in a volatile solvent and containing 5-30% of a partially polymerized resin prepared by condensing 1 molecular proportion of phenol with from 0.15 to 1.0 molecular proportion of urea and 3-5 molecular proportions of formaldehyde, said resin being soluble in the solvent, susceptible of further polymerization under the influence of heat and in its further polymerized form having the property of imparting to yarn formed from said solution a high degree of resiliency, elasticity, a springy hand or feel and a yield point in the neighborhood of 1 gram per denier.

JOHN R. CALDWELL.